

# UNITED STATES PATENT OFFICE.

OTTO RUDOLF DANIEL WITT, OF HAMBURG, GERMANY.

## METHOD OF PRODUCING TRANSPARENT CAMPHOR IN SHAPED PIECES.

995,510.

Specification of Letters Patent. Patented June 20, 1911.

No Drawing.

Application filed December 17, 1910. Serial No. 597,942.

*To all whom it may concern:*

Be it known that I, OTTO RUDOLF DANIEL WITT, Ph. D., a subject of the German Emperor, and resident of Hamburg, in the 5 German Empire, have invented a new and useful Method of Producing Transparent Camphor in Shaped Pieces, of which the following is a specification.

The present invention refers to a method 10 of producing transparent blocks, plates, bars or otherwise shaped pieces of granular, pulvulent or crystalline camphor, and this method is carried out by pressing the camphor into shape in vacuum or in rarefied air.

15 I am well aware, that it is known to bring camphor into shape so as to produce transparent solid bodies by slow sublimation, however this manner of treating camphor is attended by a considerable amount of waste 20 material and requires a long space of time. It is also known to press camphor into blocks of special shape, however these blocks have a milky, dull or opaque appearance or they are interspersed with such opaque parts.

25 Now I have found out, that these drawbacks are due to air being inclosed between the particles of the camphor and that the phenomena spoken of will not arise if the pressing is carried on in vacuum.

30 Any kind of press may be used to carry

out this method as long as means are provided for to draw off air from the space, in which the pressing operation is effected. Thus presses may be used, in which the press-members (head and ram) are suitably 35 connected with a suction device or pump, or the presses may be mounted within a space from which air is constantly sucked away or which by other means is maintained at less than atmospheric pressure.

40 The temperature used may be any temperature below the melting point of the camphor, and the pressure is that ordinarily used in compressing camphor by other, old methods, that is, must be sufficient to cause 45 the camphor particles to adhere. The longer time the camphor is subjected to pressure the less will this pressure have to be, and it may vary from 50 kg. per sq. cm. 50 upward. The vacuum ranges from 600 mms. of mercury, at which there is a distinct transparency, up to complete vacuum.

I claim:

Method of producing transparent camphor in any desired shape consisting in pressing 55 the camphor in vacuum of a suitable degree.

OTTO RUDOLF DANIEL WITT.

Witnesses:

MAX KAEMPFF,  
ERNEST H. L. MUMMENHOFF.